# EUROPEAN PATENT SPECIFICATION

(11) **EP 1 042 556 B1**
(45) Date of publication and mention of the grant of the patent: **12.05.2010**
(21) Application number: 98964756.5
(22) Date of filing: 17.12.1998
(51) Int. Cl.: D21H 17/00

(54) **PAPER PRODUCTS AND METHODS FOR APPLYING CHEMICAL ADDITIVES TO CELLULOSIC FIBERS**
PAPIERPRODUKTE UND VERFAHREN ZUM AUFTRAGEN VON CHEMISCHEN ZUSATZSTOFFEN AUF ZELLSTOFFFASERN
PRODUITS DE PAPIER ET PROCEDES POUR L'APPLICATION D'ADDITIFS CHIMIQUES SUR DES FIBRES CELLULOSIQUES

(30) Priority: 24.12.1997 US 71468 P; 22.01.1998 US 10675
(43) Date of publication of application: 11.10.2000
(73) Proprietor: KIMBERLY-CLARK WORLDWIDE, INC., Neenah, WI 54956 (US)
(72) Inventor: GOULET, Mike, Thomas, Neenah, Wisconsin 54956 (US); GEORGER, Jill, A., Neenah, WI 54956 (US); POLDERMAN, Denise, Alice, Roswell, Georgia 30076 (US); WYATT, Maurice, Alan, Evans, GA 30809 (US)
(74) Representative: Mabey, Katherine Frances
(86) International application number: PCT/US1998/026834
(87) International publication number: WO 1999/034057

(56) References cited:
- EP-A2- 0 226 408
- WO-A1-95/20066
- WO-A1-98/16570

## Description

### Background of the Invention

The present invention relates generally to paper products. More particularly, the invention concerns methods for applying chemical additives to cellulosic fibers and the paper products that can be obtained by the methods.

In the manufacture of paper products, it is often desirable to enhance physical and/or optical properties by the addition of chemical additives. Examples of properties that are developed or enhanced through the addition of chemical additives include but are not limited to dry strength, wet strength, softness, absorbency, opacity, brightness and color. During the papermaking process, chemical additives are commonly added to fiber slurries in the wet end, before the fibers are formed into a web, dewatered and dried. Traditionally, wet end additives are added to a fiber slurry that is between 0.5 and 5 percent consistency. The slurry may then be further diluted in the papermaking process before a final dilution oat the fan pump to the ultimate forming consistency.

Wet end chemical addition has several advantages over topical spray, printing or size press chemical addition methods. For instance, wet end chemical addition provides a uniform distribution of chemical additives on the fiber surfaces. Additionally, wet end chemical addition allows a selected fiber fraction to be treated with a specific chemical additive in order to enhance the performance of the paper and/or the effectiveness of the chemical additive. Further, wet end chemical addition enables multiple chemistries to be added to a fiber slurry, either simultaneously or sequentially, prior to formation of the paper web.

EP 0226408 discloses a process in which a solve is applied to a formed web to increase the rate of water removal from the web.

US 4969976 discloses a method for making dry market pulp.

One difficulty associated with wet end chemical additions is that the water soluble or water dispersible chemical additives are suspended in water and are not completely absorbed onto the cellulosic fibers. To improve adsorption of wet end additives, chemical additives are often modified with functional groups to impart an electrical charge in water. The electrokinetic attraction between charged additives and the anionically charged fiber surfaces aids the deposition and retention of chemical additives onto the fibers. Nevertheless, the amount of chemical additive that can be retained in the wet end generally follows an adsorption curve exhibiting diminishing effectiveness, similar to that described by Langmuir. As a result, the adsorption of water soluble or water dispersible chemical additives may be significantly less than 100 percent, particularly when trying to achieve high chemical additive loading levels.

Consequently, at any chemical addition level, and particularly at high addition levels, only a fraction of the chemical additive is retained on the fiber surface. The remaining fraction of the chemical additive remains dissolved or dispersed in the suspending water phase. These unadsorbed chemical additives can cause a number of problems in the papermaking process. The exact nature of the chemical additive will determine the specific problems that may arise, but a partial list of problems that may result from unadsorbed chemical additives includes: foam, deposits, contamination of other fiber streams, poor fiber retention on the machine, compromised chemical layer purity in multilayer products, dissolved solids build-up in the water system, interactions with other process chemicals, felt or fabric plugging, excessive adhesion or release on dryer surfaces, physical property variability in the finished product, and the like.

Therefore, what is lacking and needed in the art is a method for applying adsorbable chemical additives onto cellulosic fiber surfaces in the wet end of the papermaking process such that the amount of unadsorbed chemical additives in the process water is reduced or eliminated. The method minimizes the associated manufacturing and finished product quality problems that would otherwise occur.

### Summary of the Invention

It has now been discovered that chemical additives can be adsorbed onto cellulosic papermaking fibers at high levels with a minimal amount of unadsorbed chemical additives present in the papermaking process water. This is accomplished by treating a fiber slurry with an excess of the chemical additive, allowing sufficient residence time for adsorption to occur, filtering the slurry to remove unadsorbed chemical additives, and redispersing the filtered pulp with fresh water. Because the filtrate from the thickness process contains unadsorbed chemical additive, it is not sent forward in the process with the chemically treated fibers. Rather, the filtrate may be sent to the sewer or reused in a processing step prior to the filtratation step.

The present invention provides a method for applying chemical additives to cellulosic fibers in accordance with claim 1.

The invention provides a method for applying chemical additives to cellulosic fibers. The method comprises the steps of: creating a fiber slurry comprising water, cellulosic fibers, and an adsorbable chemical additive; dewatering the fiber slurry to remove unadsorbed chemical additive; and redispersing the fibers with fresh water. This method for processing cellulosic papermaking fibers enables chemical additives to be adsorbed by fibers while at the same time maintaining significantly lower levels of unadsorbed chemical additive in the water phase compared to traditional wet end chemical addition. Thus, higher concentrations of the chemical additive on the fiber relative to the process water can be achieved as compared to what has been possible with prior methods.

For purposes of the present invention, the term "cellulosic" refers to papermaking fibers comprising an amorphous carbohydrate polymer, in contrast to synthetic fibers. The term "adsorbable" is used herein to refer to a chemical additive that can be assimilated by the surface of a cellulosic fiber, in the absence of any chemical reaction involving the chemical additive and the cellulosic fiber. The term "unadsorbed" refers to any portion of the chemical additive that is not adsorbed by the fiber and thus remains suspended in the process water. The term "fresh water" is used herein to refer to water that is substantially free of the unadsorbed chemical additive. Most desirably, the fresh water is completely free of the chemical additive.

The fiber slurry is desirably dewatered to increase the consistency of the fiber slurry to about 20 percent or greater, and particularly to about 30 percent or greater, In order to remove the majority of the water containing the unadsorbed chemical additive. The fibers are thereafter redispersed, desirably to decrease the consistency of the fiber slurry to a level suitable for papermaking, to about 20 percent or less, and more particularly to about 5 percent or less, such as about 3 to about 5 percent.

The present method allows for the production of fiber furnishes that are useful for making paper products, and particularly layered paper products. Thus, the invention may provide a fiber furnish that has a higher chemical additive loading than could otherwise be achieved in combination with the relatively low level of unadsorbed chemical additive in the water. This is because chemical additive loading via traditional wet end addition is often limited by the level of unadsorbed chemical and its associated processing difficulties such as foam, deposits, chemical interactions, felt plugging, excessive dryer adhesion or release or a variety of paper physical property control issues caused by the presence of unadsorbed chemical in the water.

In one embodiment, a fiber furnish of the present invention comprises water, cellulosic fibers, and an adsorbable chemical additive. The amount of chemical additive adsorbed onto the fibers is about 2 kilograms per metric ton or greater, and the amount of unadsorbed chemical additive in the water is between 0 and about 20 percent of the amount of chemical additive adsorbed onto the fibers. In particularly desirable embodiments, the amount of adsorbed chemical additive is about 3 kg/metric ton or greater, particularly about 4 kg/metric ton or greater, and more particularly about 5 kg/metric ton or greater. Moreover, the amount of unadsorbed chemical additive in the water is between 0 and about 15 percent, particularly between 0 and about 10 percent, and more particularly between 0 and about 7 percent, of the amount of adsorbed chemical additive.

Another aspect of the invention resides in a method for making chemically treated paper products. The method comprises the steps of: creating a first fiber slurry comprising water, cellulosic fibers, and an adsorbable chemical additive; creating a second fiber slurry that is substantially free of the adsorbable chemical additive; dewatering the first fiber slurry to remove unadsorbed chemical additive; redispersing the fibers in the first fiber slurry with fresh water; and forming a paper product using a layered headbox, the first fiber slurry supplied to a first headbox layer and the second fiber slurry supplied to a second headbox layer.

In another embodiment, a method for making a paper product comprises the steps of: creating a fiber slurry comprising water, cellulosic fibers and a first adsorbable chemical additive; dewatering the fiber slurry to a consistency of about 20 percent or greater; passing the dewatered fiber slurry through a disperser to mechanically work the fibers; diluting the fiber slurry with fresh water that is substantially free of the first chemical additive to a consistency of about 5 percent or less; adding a second adsorbable chemical additive comprising a debonding agent or a softening agent to the fiber slurry; dewatering the fiber slurry to a consistency of about 20 percent or greater; diluting the fiber slurry with fresh water that is substantially free of the second chemical additive to a consistency of about 5 percent or less; and forming a paper product from the fiber slurry. The first chemical additive may comprise, for example, a bonding agent to decrease the amount of lint from the product.

The present invention is particularly useful for adding chemical additives such as softening agents and debonding agents to the outer layer furnishes in a three layer paper product. In particular tissue products, for example, the center layer is adapted to provide strength development and control. The present invention allows the softening agents and debonding agents to be applied to the outer layers while minimizing contamination of the center strength layer.

Hence, another aspect of the invention resides in paper products formed from fibers that have been chemically treated to minimize the amount of residual, unadsorbed chemical additives in the process water. These paper products exhibit high chemical "purity" on the fiber fraction that has been treated using the present method and offer the ability to achieve excellent chemical layer purity when using a stratified headbox and/or the ability to achieve fiber specific chemical treatment in papers made from blends of two or more fiber types. The term "paper" is used herein to broadly include writing, printing, wrapping, sanitary, and industrial papers, newsprint, linerboard, tissue, napkins, wipers, towels, or the like.

The chemical additives that can be used in conjunction with the present invention include: dry strength aids, wet strength aids, softening agents, debonding agents, absorbency aids, sizing agents, dyes, optical brighteners, chemical tracers, opacifiers, dryer adhesive chemicals, and the like. Additional forms of chemical additives may include: pigments, emollients, humectants, viricides, bactericides, buffers, waxes, fluoropolymers, odor control materials and deodorants, zeolites, perfumes, debonders, vegetable and mineral oils, humectants, sizing agents, superabsorbents, surfactants, moisturizers, UV blockers, antibiotic agents, lotions, fungicides, preservatives, aloe-vera extract, vitamin E, or the like. Suitable chemical additives are adsorbable by the cellulosic Papermaking fibers and are water soluble or water dispersible.

The term "softening agent" refers to any chemical additive that can be incorporated into paper products such as tissue to provide improved tactile feel. These chemicals can also act as debonding agents or can act solely to improve the surface characteristics of tissue, such as by educing the coefficient of friction between the tissue surface and the hand.

The term "debonding agent" refers to any chemical that can be incorporated into paper products such as tissue to prevent or disrupt interfiber or intrafiber hydrogen bonding. Depending on the nature of the chemical, debonding agents may also act as softening agents. In contrast, the term "bonding agent" refers to any chemical that can be incorporated into tissue to increase or enhance the level of interfiber or intrafiber bonding in the sheet. The increased bonding can be either ionic, Hydrogen or covalent in nature.

The term "water soluble" refers to solids or liquids that will form a solution in water, and the term "water dispersible" refers to solids or liquids of colloidal size or larger that can be dispersed into an aqueous medium.

The method for applying chemical additives to papermaking fibers may be used in a wide variety of papermaking operations, including wet pressing and creped or uncreped throughdrying operations. By way of illustration, various tissue making processes are disclosed in U.S. Patent 5,667,636 issued September 16, 1997 to S. A. Engel et al.; and U.S. Patent 5,607,551 issued March 4, 1997 to T. E. Farrington, Jr. et al.

The method may also be used in alternative processes, including: chemically pretreating pulp in a pulp mill before a dry lap machine or crumb baler; adding chemical additives in sequence to reduce interactions; removing chemical additives from a fiber slurry (neutralizing anionic components, sizing or softening formulations) after a chemical additive has been added to facilitate the removal process; or the like.

Many fiber types may be used for the present invention including hardwood or softwoods, straw, flax, milkweed seed floss fibers, abaca, hemp, kenaf, bagasse, cotton, reed, and the like. All known papermaking fibers may be used, including bleached and unbleached fibers, fibers of natural origin (including wood fiber and other cellulosic fibers, cellulose derivatives, and chemically stiffened or crosslinked fibers), some component portion of synthetic fibers (synthetic papermaking fibers include certain forms of fibers made from polypropylene, acrylic, aramids, acetates, and the like), virgin and recovered or recycled fibers, hardwood and softwood, and fibers that have been mechanically pulped (e.g., groundwood), chemically pulped (including but not limited to the kraft and sulfite pulping processes), thermomechanically pulped, chemithermomechanically pulped, and the like. Mixtures of any subset of the above mentioned or related fiber classes may be used. The fibers can be prepared in a multiplicity of ways known to be advantageous in the art. Useful methods of preparing fibers include dispersion to impart curl and improved drying properties, such as disclosed in U.S. Patents 5,348,620 issued September 20, 1994 and 5,501,768 issued March 26, 1996, both to M. A. Hermans et al. and U.S. Patent 5,656,132 issued August 12, 1997 to Farrington, Jr. et al.

A single headbox or a plurality of headboxes may be used. The headbox or headboxes may be stratified to permit production of a multilayered structure from a single headbox jet in the formation of a web. In particular embodiments, the web is produced with a stratified or layered headbox to preferentially deposit shorter fibers on one side of the web for improved softness, with relatively longer fibers on the other side of the web or in an interior layer of a web having three or more layers. The web is desirably formed on an endless loop of foraminous forming fabric which permits drainage of the liquid and partial dewatering of the web. Multiple embryonic webs from multiple headboxes may be couched or mechanically or chemically joined in the moist state to create a single web having multiple layers.

Numerous features and advantages of the present invention will appear from the following description. In the description, reference is made to the accompanying drawings which illustrate preferred embodiments of the invention. Such embodiments do not represent the full scope of the invention. Reference should therefore be made to the claims herein for interpreting the full scope of the invention.

### Brief Description of the Drawings

Figure 1 depicts a schematic process flow diagram of a method according to the present invention for treating papermaking fibers with chemical additives.
Figure 2 depicts a schematic process flow diagram of a method according to the present invention for both treating papermaking fibers with chemical additives and mechanically treating the fibers using a disperser.
Figure 3 depicts a schematic process flow diagram for a method of making an uncreped tissue sheet.

### Detailed Description of the Drawings

The invention will now be described in greater detail with reference to the Figures. For simplicity, the various tensioning rolls schematically used to define the several fabric runs are shown but not numbered, and similar elements in different Figures have been given the same reference numeral. A variety of conventional papermaking apparatuses and operations can be used with respect to the stock preparation, headbox, forming fabrics, web transfers, creping and drying. Nevertheless, particular conventional components are illustrated for purposes of providing the context in which the various embodiments of the invention can be used.

Figure 1 depicts stock preparation equipment used to apply chemical additives to papermaking fibers according to one embodiment of the present invention. The stock preparation equipment comprises a first stock chest 10, a second stock chest 12, and a dewatering device 14 operably disposed between the stock chests. Papermaking fibers and water are added to the first stock chest 10 to form a fiber slurry 20. The fiber slurry in the first stock chest desirably has a consistency of about 20 percent or lower, and particularly about 5 percent or lower, such as about 3 to about 5 percent. The fiber slurry in the first stock chest is desirably under agitation using a mixing blade, rotor, recirculation pump, or other suitable device 18 for mixing the fiber slurry.

One or more chemical additives 24 are supplied from a reservoir 26 and added to the fiber slurry 20 in the first stock chest 10. The amount of chemical additive 24 is suitably about 5 to about 20 kg./metric ton. In particular embodiments, the chemical additive comprises an imidazoline-based debonding agent and is added in an amount from about 7.5 to about 15 kg./metric ton. The fiber slurry and chemical additive are desirably allowed to remain together in the first stock chest under agitation for a residence time sufficient to allow the papermaking fibers to adsorb a substantial portion of the chemical additive 24. A residence time of about 15 to about 30 minutes, for instance, may be sufficient.

The fiber slurry 20 is thereafter transferred through suitable conduits 27 and a pump 28 to the dewatering device 14. In the illustrated embodiment, the dewatering device comprises a belt press 14, although alternative dewatering devices such as a centrifuge, a nip thickening device or the like may be used. The fiber slurry is injected between a pair of foraminous fabrics 30 such that press filtrate 32 is removed from the slurry. The press filtrate 32 comprises a portion of the process water along with unadsorbed chemical additives 24 in the water. The belt press 14 or other dewatering device suitably increases the fiber consistency of the slurry to about 20 percent or greater, and particularly about 30 percent or greater. The unadsorbed chemical additive can be removed from the process or used as dilution water in prior stock preparation steps, but importantly it is not sent forward with the chemically treated furnish.

The thickened fiber slurry 20 is then transported through conduits 34 to the second stock chest 12. The fiber slurry is then re-diluted with fresh water 35 from a suitable reservoir 36 and optionally agitated using a mixing device 18. The fiber consistency of the slurry is suitably decreased to about 20 percent or less, and particularly about 5 percent or less, such as about 3 to about 5 percent. The fiber slurry may then be removed from the second stock chest through suitable conduits 37 and a pump 38 for subsequent processing 39. Alternatively, the fiber slurry may be processed through the foregoing procedure again in an effort to further increase the chemical additive retention level.

Figure 2 depicts an alternative embodiment of the present invention in which stock preparation equipment is used to apply chemical additives to papermaking fibers and to mechanically treat the fibers. In general, the equipment comprises three stock chests 10, 12 and 40, two dewatering devices 14 and 42, two dilution water chests 44 and 46, and a disperser 48 for mechanically treating the papermaking fibers.

Papermaking fibers and water are added to the first stock chest 10 to form a fiber slurry 20. The fiber slurry in the first stock chest desirably has a consistency of about 20 percent or lower, and particularly about 5 percent or lower. One or more chemical additives 24 are supplied from a reservoir 26 and added to the fiber slurry 20 in the first stock chest 10 while under agitation 18. The first chemical additive added to the fiber slurry is desirably a cationic bonding agent which is used to control lint in the finished product. The first chemical additive is desirably not a softening agent or debonding agent that would reduce the efficiency of the disperser.

After a sufficient residence time, the fiber slurry is transferred through suitable conduits 27 and a pump 28 to a belt press 14 or other suitable dewatering device. Unadsorbed chemical additives in the water are removed with the press filtrate 32 during the pressing operation and stored in the first dilution water chest 44. The contents of the first dilution water chest may be used as either pulper make-up water or dilution water or may be discarded. The dewatering device 14 suitably increases the fiber consistency of the slurry to about 20 percent or greater, and particularly about 30 percent or greater.

The thickened fiber slurry 20 is then transported through suitable conduits 34 to the disperser 48 for mechanical treatment of the fibers. Dispersers suitable for use in the present method are disclosed in U.S. Patents 5,348,620 issued September 20, 1994 and 5,501,768 issued March 26, 1996, both to M. A. Hermans et al.

After dispersing, the fiber slurry is transported via conduits 50 to the second stock chest 12. A second chemical additive or second group of chemical additives 52 are supplied from a reservoir 53 and added to the fiber slurry 20 in the second stock chest 12 while under agitation 18. Additionally, the fiber slurry may optionally be diluted with filtrate 56 from a source described hereinafter. The fiber consistency of the slurry is suitably decreased to about 20 percent or lower, and particularly about 5 percent or lower, such as about 3 to about 5 percent. In particular embodiments, the second chemical additive 52 comprises a softening agent and/or a debonding agent, and the fiber slurry is not subjected to high shear refining forces such as those generated in a disperser once the softening and/or debonding agent is added to the fiber slurry.

After a sufficient residence time to permit adsorption of the second chemical additive, the fiber slurry 20 is transferred from the second stock chest 12 through suitable conduits 58 and a pump 59 to the second dewatering device 42. Unadsorbed portions of the second chemical additive 52 in the water are removed with the press filtrate 56 during the pressing operation and stored in the second dilution water chest 46. The contents of the second dilution water chest may be added to the second stock chest 12 as described above or may be discarded. The second dewatering device 42 suitably increases the fiber consistency of the slurry to about 20 percent or greater, and particularly about 30 percent or greater.

The thickened fiber slurry 20 is then transported through conduits 58 to the third stock chest 40. The fiber slurry is then re-diluted with fresh water 35 from a suitable reservoir 36 and optionally agitated using a mixing device 18. The fiber consistency of the slurry is suitably decreased to about 20 percent or lower, and particularly about 5 percent or lower, such as about 3 to about 5 percent. The fiber slurry may then be removed from the third stock chest through suitable conduits 37 and a pump 38 for subsequent processing 39. Alternatively, the fiber slurry may be returned to the second stock chest 12 for repeated application of the second chemical additive 52.

One suitable process 39 for making paper products from the fiber slurries 20 of Figures 1 or 2 is the uncreped throughdrying method depicted in Figure 3. The uncreped throughdrying method is also disclosed in U.S. Patent 5,656,132 issued August 12, 1997 to Farrington, Jr. et al. A twin wire former having a layered papermaking headbox 60 injects or deposits a stream from the fiber slurry 20 onto the forming fabric 62 to form a cellulosic web 64. The web is then transferred to fabric 66, which serves to support and carry the newly-formed wet web downstream in the process as the web is partially dewatered to a consistency of about 10 dry weight percent. Additional dewatering of the wet web can be carried out, such as by vacuum suction, while the wet web is supported by the forming fabric.

The wet web is then transferred from the forming fabric 66 to a transfer fabric 70 traveling at a slower speed than the forming fabric in order to impart increased MD stretch into the web. A kiss transfer is carried out to avoid compression of the wet web, preferably with the assistance of a vacuum shoe 72. The transfer fabric can be a fabric having impression knuckles or it can be a smoother fabric such as Asten 934, 937, 939, 959 or Albany 94M. If the transfer fabric is of the impression knuckle type described herein, it can be utilized to impart some of the same properties as the throughdrying fabric and can enhance the effect when coupled with a throughdrying fabric also having the impression knuckles. When a transfer fabric having impression knuckles is used to achieve the desired CD stretch properties, it provides the flexibility to optionally use a different throughdrying fabric, such as one that has a decorative weave pattern, to provide additional desirable properties not otherwise attainable.

The web is then transferred from the transfer fabric to a throughdrying fabric 74 with the aid of a vacuum transfer roll 76 or a vacuum transfer shoe. The throughdrying fabric can be traveling at about the same speed or a different speed relative to the transfer fabric. If desired, the throughdrying fabric can be run at a slower speed to further enhance MD stretch. Transfer is preferably carried out with vacuum assistance to ensure deformation of the sheet to conform to the throughdrying fabric, thus yielding desired bulk, flexibility, CD stretch and appearance. The throughdrying fabric is preferably of the impression knuckle type.

The level of vacuum used for the web transfers can be from about 3 to about 15 inches (about 75 to about 380 millimeters) of mercury, preferably about 10 to about 15 inches (about 254 to about 380 millimeters) of mercury. The vacuum shoe (negative pressure) can be supplemented or replaced by the use of positive pressure from the opposite side of the web to blow the web onto the next fabric in addition to or as a replacement for sucking it onto the next fabric with vacuum. Also, a vacuum roll or rolls can be used to replace the vacuum shoe(s).

Specific embodiments and modes of operation relating to the forming fabric, transfer fabric, rush transfer, transfer shoes, fabric positioning, and vacuum levels are disclosed in U.S. Patent 5,667,636 issued September 16, 1997 to S. A. Engel et al. and U.S. Patent 5,607,551 issued March 4, 1997 to T. E. Farrington, Jr. et al.

While supported by the throughdrying fabric, the web is final dried to a consistency of about 94 percent or greater by the throughdryer 80 and thereafter transferred to a carrier fabric 82. The dried basesheet is transported to the reel 84 using carrier fabric 82 and an optional carrier fabric 86. An optional pressurized turning roll 88 can be used to facilitate transfer of the web from carrier fabric 82 to fabric 86. Suitable carrier fabrics for this purpose are Albany International 84M or 94M and Asten 959 or 937, all of which are relatively smooth fabrics having a fine pattern. The roll of tissue may then be calendered, slit, surface treated with emollient or softening agents, embossed, or the like in subsequent operations to produce the final product form.

### EXAMPLES

The following examples serve to illustrate possible approaches pertaining to the present invention. The particular amounts, proportions, compositions and parameters are meant to be exemplary, and are not intended to specifically limit the scope of the invention.

### Example 1 (Comparative)

For this example, a softening/debonding agent was added during production of a multi-fiber, three-layer tissue using a conventional, stuffbox chemical addition method. The furnish used for the outer two layers comprised 70% Eucalyptus fibers, 29% tissue broke and 1% recycled fiber corestock. The outer layer furnish components were blended at the pulper. After repulping, the furnish was transferred to a chest and treated with a bonding agent, Parez 631 NC which is commercially available from Cytec Industries, Inc., at a dosage of 1 kg./metric ton. After allowing the slurry to mix for 20 minutes, the furnish was thickened to greater than 30% consistency using a dewatering press and treated in a disperser to impart curl to the fibers. The disperser was operated with a power input of 80 kilowatts and an exit stock temperature of about 82.2°C (180°F). After dispersing, the fibers were stored in a high density chest until needed during tissue manufacturing.

At the time of manufacturing, the outer layer furnish, consisting of the dispersed Eucalyptus/broke/corestock blend, was diluted to 3.5% consistency in a chest using the filtrate from the earlier thickness process. A softening/debonding agent, C-6092 which is commercially available from Witco Corp., was added to this furnish at a rate of 6.5 kg./metric ' ton at the machine chest stuffbox recirculation loop. This stuffbox feeds the fan pumps for both outer layers of a three-layer tissue sheet.

The center layer furnish comprised 100% northern bleached softwood kraft fibers. This furnish was refined at an energy input of 2 horsepower days^{a}/metric ton for dry strength development. Parez 631 NC was also added to this furnish at a dosage of 5.8 kg./metric ton to achieve wet tensile strength control. Dry strength control was achieved by varying the ratio of center layer to outer layer furnish.
^{a}1 horsepower day - 64 MJ

A one-ply, uncreped through air dried tissue was produced using a pilot tissue machine. This same tissue machine was used for Examples 1-4. The machine contains a 3 layer headbox, of which the outer layers contain the same furnish (70% Eucalyptus, 29% broke, 1% corestock) and the center layer was 100% softwood fiber. The resulting three-layered sheet structure was formed on a twin-wire, suction form roll, former. The speed of the forming fabrics was 1143 cm per sec. (2250 feet per minute) (fpm). The newly-formed web was then dewatered to a consistency of about 20-27 percent using vacuum suction from below the forming fabric before being transferred to the transfer fabric, which was travelling (914 cm/sec (1800 feet per minute) (25% rush transfer). A vacuum shoe pulling about 25.4 cm (10 inches) of mercury vacuum was used to transfer the web to the transfer fabric. The web was then transferred to a throughdrying fabric travelling at a speed of about 914 cm/sec (1800 fpm). The web was carried over a pair of Honeycomb throughdryers operating a temperatures of about 163°C (325°F) and dried to final dryness of about 94-98 percent consistency.

The air dry basis weight of the sheet was 27.5 gsm. The final fiber ratio in the sheet was 32% softwood fiber (in center layer) and 68% Eucalyptus/broke/corestock blend (outer layers). The final strength of the tissue was 800 grams per 7.62 cm (3 inch) width (geometric mean tensile strength).

### Example 2

For this example, which is in accordance with the invention, the improved chemical addition method shown in Figure 1 was used to treat a furnish with a softening/debonding agent. The treated furnish was then used as the outer layer furnish in a multi-fiber, three-layered tissue structure. Because the improved chemical addition method removes most non-retained softening/debonding agent from the water phase during tissue forming, the resultant product can be produced at equivalent tensile strength, higher softener/debonder content and a lower softwood fiber content than a tissue made with the identical softening agent using the conventional chemical addition method described in Example 1.

In Example 2, the furnish used for the outer two layers comprised 70% Eucalyptus fibers, 29% tissue broke and 1% recycled fiber corestock. During the stock preparation phase, the outer layer furnish was blended during repulping and placed in a stock chest at 3.5% consistency. The furnish was then treated with a bonding agent, Parez 631 NC from Cytec Industries, Inc., at a dosage of 1 kg./metric ton. After allowing the slurry to mix for 20 minutes, a softening/debonding agent, C-6092 from Witco Corp., was added at a dosage of 7.5 kg. of active chemical/metric ton of fiber. After an additional 20 minutes of mixing time, the slurry was dewatered using a belt press to approximately 32% consistency. The filtrate from the dewatering process was used as pulper make-up water for subsequent batches but not sent forward in the stock preparation or tissuemaking process. The thickened pulp was then passed through a disperser with a power input of 80 kilowatts and a stock temperature of about 82.2°C (180°F) to impart curl to the fibers. After the dispersing operation, the stock was placed in a high density storage chest until needed during tissue manufacturing.

A one-ply, uncreped, through air dried tissue was made using a three layered headbox, as described in Example 1. The furnish for the outer two layers comprised the chemically treated 32% consistency Eucalyptus/broke/corestock furnish blend, which had been re-diluted to 3% consistency with fresh water in a chest under agitation. The center layer consisted of 100% softwood fibers refined at an energy input of 2 horsepower days/metric ton, to whcih 5.8 kg./metric ton of Parez 631 NC was added for wet strength control. Finished product dry strength control was achieved by adjusting the ratio of center layer and outer layer furnish in the sheet.

The air dry basis weight of the sheet was 27.5 gsm. The final fiber ratio in the sheet was 17% softwood fiber (in center layer) and 83% Eucalyptus/broke/corestock blend (outer layers). The final strength of the tissue was 802 grams per 7.62 cm (3 inch) width (geometric mean tensile strength).

### Example 3

For this example, the improved chemical addition method shown in Figure 2 was used to first treat a furnish with a bonding agent, mechanically modify the fibers using a disperser, and then treat the furnish with a softening/debonding agent. The chemically treated furnish was used as one furnish in a multi-fiber, three-layered tissue structure. Because the improved chemical addition method removes most non-retained softening/debonding agent from the water phase during tissue forming, the resultant product was much stronger (at equal fiber composition) than a tissue made with similar softening agent using the conventional chemical addition method described in Example 1. In addition, because the softener/debonder is not present on the furnish during the dispersing operation, there is a more efficient transfer of energy to the fibers. This results in a higher level of debonding than demonstrated in Example 2 due to the fiber curl properties imparted during dispersing.

In Example 3, the furnish used for the outer two layers comprised 70% Eucalyptus fibers, 29% tissue broke and 1% recycled fiber corestock. During the stock preparation phase, the outer layer furnish was blended during repulping and placed in a stock chest at 3.5% consistency. The furnish was then treated with a bonding agent, Parez 631 NC from Cytec Industries, Inc., at a dosage of 1 kg./metric ton. After allowing the slurry to mix for 20 minutes, the furnish was dewatered using a belt thickening press to greater than 30% consistency. The thickened pulp was then passed through a disperser with a power input of 80 kilowatts and a stock temperature of about 82.2°C (180°F) to impart curl to the fibers. The high consistency, dispersed pulp was then stored in a chest until sufficient quantities could be produced. This method is not in accordance with the present invention in which the adsorbable chemical additive is added to the slurry of water and cellulosic fibers in an amount of about 5 kg per metric ton or greater, but has been retained to facilitate understanding of the invention.

In order to treat the furnish with a second chemical additive, the high consistency pulp was then diluted to 3.5% consistency with a combination of fresh water and thickener filtrate (containing unadsorbed softening/debonding agent, as shown in Figure 2). The furnish was next treated with 7.5 kg./metric ton of a softening/debonding agent, C-6092 from Witco Corp., and allowed to mix for 20 minutes. The furnish was then dewatered using a belt press to approximately 32% consistency. The filtrate from the dewatering process was used as partial dilution water for the high consistency stock dilution step, as previously mentioned. After the second thickening operation, the stock was placed in a high density storage chest until needed during tissue manufacturing.

A one-ply, uncreped, through air dried tissue was made using a three layered headbox, as described in Example 1. The furnish for the outer two layers comprised the chemically treated 32% consistency Eucalyptus/broke/corestock furnish blend, which had been re-diluted to 3% consistency with fresh water in a chest under agitation. The center layer comprised 100% softwood fibers refined at an energy input of 2 horsepower^{b} days/metric ton, to which 5.8 kg./metric ton of Parez 631 NC was added for wet strength control. Finished product dry strength control was achieved by adjusting the ratio of center layer and outer layer furnish in the sheet.
^{b}1 horsepower day - 64 MJ

The air dry basis weight of the sheet was 27.5 gsm. The final fiber ratio in the sheet was 24% softwood fiber (in center layer) and 76% Eucalytpus/broke/corestock blend (outer layers). The final strength of the tissue was 806 grams per 7.62 cm (3 inch) width (geometric mean tensile strength).

### Example 4

This example is similar to Example 3, except that 15 kg./metric ton of C-6092 softener/debonder was added to the outer layer furnish (instead of 7.5 kg./metric tone in Example 3). Because the improved chemical addition method has removed most non-retained softening/debonding agent from the water phase during tissue formation, the resultant product contains 55% more softening/debonding agent than the product described in Example 1, at equivalent tensile strength and fiber composition.

The stock preparation and tissue manufacturing procedures were identical to Example 3. The air dry basis weight of the sheet was 27.5 gsm. The final fiber ratio in the sheet was 31% softwood fiber (in center layer) and 60% Eucalyptus/broke/corestock blend (outer layers). The final strength of the tissue was 795 grams per 7.62 cm (3 inch) width (geometric mean tensile strength).

The results shown in Table 1 below indicate that a layered tissue sheet can be made with a geometric mean tensile strength of about 800 grams per 7.62 cm (3 inch) width (795 grams per 3 inch width), under the processing conditions described in Exmaple 5, that contains 31% softwood fiber and 5.9 kg./metric ton of retained C-6092 softener/debonder by using the improved chemical addition method. When using the conventional chemical addition method described in Example 1, and otherwise identical manufacturing conditions, a layered tissue sheet with a geometric mean tensile strength of 800 g./7.62 cm/(3") width contains 32% softwood fiber but only 3.8 kg./metric ton of retained C-6092 softener/debonder. The reason for this difference in retained C-6092 at equivalent tissue strength, it is hypothesized, is because the debonding characteristic of the unadsorbed C-6092 in the conventional chemical addition method compromises the strength development of the softwood fibers in the center layer. As a result, more softwood fiber is need to achieve the same finished product tensile strength.

By using the improved chemical addition method, tissue fiber/chemistry combinations can be produced at target strength levels that could not otherwise be made using conventional chemical addition methods. In Examples 2-4, the tissues were manufactured with generally constant basis weight and strength by adjusting the relative amounts of softwood and hardwood. Of course, various alternatives are possible such as maintaining generally constant strength and softwood/hardwood proportion and adjusting the basis weight.

**TABLE 1**

| Examples 1 - 4 | | | | | |
|---|---|---|---|---|---|
| Example | Strength g./7.62 cm (3") | % Center Layer | % Outer Layer | Debonder Add-on | Debonder Retained |
| 1 | 800 | 32 | 68 | 4.4 | 3.8 |
| 2 | 802 | 17 | 83 | 6.2 | 4.6 |
| 3 | 806 | 24 | 76 | 5.7 | 3.8 |
| 4 | 795 | 31 | 69 | 10.4 | 5.9 |

In Table 1, "Strength" refers to the geometric mean tensile strength which is calculated for purposes of the present invention according to the formula:
$\sqrt{\left[\left(MDtensile\right)⁢\left(CDtensile\right)\right]} .$ The "MD tensile" strength of a tissue sample is the conventional measure, known to those skilled in the art, of load per sample width at the point of failure when a tissue web is stressed in the machine direction. Likewise, "CD tensile" strength is the analogous measure taken in the cross-machine direction MD and CD tensile strength are measured using an Instron tensile tester using a 3-inch^{c} jaw width, a jaw span of 4 inches^{c}, and a crosshead speed of 10 inches^{c} per minute. Prior to testing the sample is maintained under TAPPI conditions (22.8°C (73°F), 50% relative humidity) for 4 hours before testing. Tensile strength is reported in units of grams per 3 inch^{c} width (at the failure point).
   ^{c} 1 inch = 2.54 cm.

The % Center Layer and % Outer Layer refer to the weight percent of fibers in the appropriate layers.

The Debonder Add-on reflects the chemical additive that is added to the furnish in kg./metric ton of the entire sheet. This is calculated based on the add-on level to the outer layer furnish and the amount of the outer layer furnish in the final sheet.

The Debonder Retained reflects the amount of chemical additive adsorbed onto the tissue. The Debonder Retained can be determined using the following procedure suitable for imidazoline-based chemical additives such as Witco C-6092 that are added to the tissue. The procedure references the percent add-on, which has been converted to kg./metric ton (multiplied by 10) in Table 1. In general, a sample of the tissue is weighed and extracted in a sealed container for a given amount time on a flatbed shaker at ambient conditions. After the extraction, the tissue is removed and the extract allowed to settle. The extract is then analyzed by ultraviolet spectrometer. After the percent extracted is calculated, the add-on percent can be determined by reference to an add-on correlation curve that is generated as described below.

The following equipment and chemicals are used: pipets, 1, 3, 5, 10 and 100 mL; volumetric flasks, 100 and 1000 mL; sealed containers, e.g. specimen cups; a flatbed shaker, such as an orbital flatbed shaker (Lab Line Orbital Shaker Model No. 3590, Lab Line Instruments, Inc.); an ultraviolet spectrometer (Hewlett Packard Model 8451A Diode Array Spectrophotometer, Hewlett Packard); methanol, reagent grade; imidazoline, standard such as Witco C-6092; beakers, 30 mL; and control tissues that differ from the tissue being tested only by the absence of the chemical additive being tested.

A stock standard imidazoline solution (1000 ppm active) is prepared: Weigh 0.1250 grams of C-6092 (80% active) into a 30mL beaker; transfer quantitatively to a 100mL flask with methanol; and dilute to mark with methanol and invert several times.

Standard imidazoline solutions (10, 30, 50, 100 ppm) are prepared: Into four 100 mL volumetric flasks, add 1, 3, 5, and 10 mL of the 1000 ppm stock standard imidazoline solution; and dilute to marks with methanol. The standards are 10, 30, 50 and 100 ppm, respectively.

Generate a Standard Solution Curve: With the UV spectrophotometer set at 238 nm wavelength, reference the instrument using a methanol sample. Read the absorptance of the standard solutions (10, 30, 50 and 100 ppm), then plot a curve of the concentration versus absorptance. Generate a first-order equation fit of the data.

Spiking solutions (1000 and 5000ppm) are prepared: Weigh out 1.250 and 6.250 grams of C-6092 into 50 ml beakers; transfer quantitatively to a 1000 ml flask with distilled water; shake well and allow to dissolve before diluting to mark. If excessive foaming occurs, fill to the stem of the flask and add a small amount of methanol to eliminate the foam and dilute to mark then invert several times. This makes a 1000 ppm and 5000 ppm spiking solutions.

Generate an Add-On Correlation Curve: A minimum of three replicates should be performed for each level of add-on and for blanks. There should be at least four levels of add-on to generate a curve. Spiking solutions should be made with distilled water, so that the spiked sample can be dried in a 60 degree Celsius oven.

Weigh out 5.00 grams of control tissue into a specimen container. For four levels, three replicates, and blanks, prepare 15 samples. A typical curve would be 0.1, 0.3, 0.8, and 1.0% C-6092 add-on based on the weight of the tissue.

Spike samples with spiking solution and dry for 48 hours in a 60 degree Celsius oven. Use volumetric pipettes. Example:

| | Volume of Spiking Solution for 5.00 gram tissue | |
|---|---|---|
| Add-on Level | 1000ppm | 5000ppm |
| Blank | 0 mL | 0 mL |
| 0.1% | 5 mL | --- |
| 0.3% | 15 mL | --- |
| 0.8% | --- | 8 mL |
| 1.0% | --- | 10 mL |

Add 100 mL of methanol using a pipet and seal the containers. Place in a flatbed shaker and extract for ½ hour. Remove tissue and allow the extract to settle. With a transfer pipette, remove supernatant and fill a spectrophotometer cuvette. Measure the absorptance at 238nm wavelength using the UV spectrometer. A 1 to 10 dilution may be required to stay within the standard curve. Blanks should be read with and without this dilution. Subtract the mean absorptance readings from the blanks. Use the 1/10 dilution blank readings for 1/10 dilution samples and no dilution blank readings for the no dilution samples.

The percent extracted is then calculated from the ppm reading from the standard curve (imidazoline) as follows: $% Extracted \left(no dilution\right) = ppm reading \times 0.1 \times 100 / 5000.$ $% Extracted \left(1/10 dilution\right) = ppm reading \times 0.1 \times 10 \times 100 / 5000.$

Construct an Add-on Correlation curve with the percent extracted values (y-axis) versus the corresponding add-on level (x-axis). Select the best fitting curve (first or second order).

Sample Analysis: Weigh out 5.00 grams sample in a specimen container and add 100 mL of methanol. Place on the flatbed shaker and extract for ½ hour. Remove the tissue and allow to settle. Read the extracts at 238nm wavelength and subtract the mean blank absorptance reading. Calculate the ppm from the standard curve and then calculate the percent extracted value. Using the Add-on correlation curve, calculate the percent add-on with the percent extracted value.

Imidazoline has a peak absorptance at 238nm wavelength. While blank tissue extracts do not have this peak absorptance at 238nm, it does have some absorptance that interferes with the quantitation. Blanks are quite reproducible and can be subtracted for the determination. It is important that the weight of the sample, volume of methanol, and the extraction time be kept constant. An add-on correlation curve should be generated for different tissue samples, because various chemicals used in the tissue process can affect the binding of the imidazoline thus affecting the recovery. Percent add-on also affects the percent recovery; using various levels of add-on in constructing the correlation curve helps to determine the add-on value.

### Example 5

To better illustrate the ability for the improved chemical addition method to remove unadsorbed chemicals from the furnish of a papermaking process, a laboratory scale experiment was conducted. The objective of this experiment was to demonstrate how much unadsorbed chemical is present in systems that do not use the improved addition method and compare this to systems in which the same amount of chemical is added using the improved method. The furnish used in this experiment was 100% Eucalyptus fibers. The chemical additive used was C-6092, a softener/debonder commercially available from Witco Corp. The addition levels were 0.5% and 1.0% active debonder on dry fiber. In accordance with the invention, adsorbable chemical additive is added to a slurry of water and cellulosic fibers in an amount of 5 kilograms per metric ton or greater.

### 0.5% Addition Experiment: Step 1

During the experiment, 1800 grams of a 2.5% consistency fiber slurry (45 g. dry fiber) were agitated using a mechanical mixer. To the fiber slurry under agitation, the appropriate amount of C-6092 chemical was added in the form of a 1% active solution. The volume of 1% active C-6092 required for a 0.5% loading was 22.5 ml. After agitation for 15 minutes, 600 ml of slurry was removed and spread out on a plate to dry at room temperature under a hood. This sample will be referred to as 1A.

### Step 2

The remaining 1200 grams of slurry were filtered using a Whatman 4 filter paper and Buchner funnel apparatus. This filtration step simulates the dewatering step of the improved chemical addition method shown in Figure 1. The filter pad (at approximately 25% consistency) was split into two sections of approximately equal mass. One section was placed in the hood to dry at room temperature. This sample will be referred to as 2A.

### Step 3

The other half of the filter pad (approximately 600 g.) was redispersed to 2.5% consistency using distilled water. The slurry was mechanically agitated for 15 minutes and then filtered using a Whatman 4 filter paper and Buchner funnel apparatus. This filtration step simulates the dewatering that occurs in the forming and vacuum dewatering zones of a tissue machine. The filter pad was placed in a hood to dry at room temperature. This sample will be referred to as 3A.

### 1.0% Addition Experiment

Steps 1 - 3 were repeated using a 1.0% addition level of C-6092. The corresponding samples were coded 1B, 2B and 3B.

All samples were analyzed for C-6092 content using a methanol extraction followed by UV spectroscopic analysis at 238nm and comparison of the absorptance to a known calibration curve. The results are shown in the table below:

| | Sample No. | | | | | |
|---|---|---|---|---|---|---|
| | 1A | 2A | 3A | 1B | 2B | 3B |
| C-6092 Content (%) | 0.51 | 0.30 | 0.28 | 1.05 | 0.73 | 0.68 |

The results demonstrate the impact of using the improved chemical addition method on reducing the amount of unadsorbed debonder in the furnish. Comparing the C-6092 content of samples 1A and 2A shows that 41% of the chemical is not retained sufficiently onto the fibers and is removed during dewatering. If the conventional stuffbox chemical addition method is used this unadsorbed chemical is free in the furnish to contaminate other fiber streams and cause the processing problems previously described. Comparing the C-6092 content of samples 2A and 3A, however, shows that only an additional 6% of the retained C-6092 is removed during a second dewatering step, which simulates sheet formation on a tissue machine.

When the C-6092 content of the 1B, 28 and 38 samples are compared it can be shown that 30% of the original 1.0% chemical loading is removed during the first dewatering step, but only an additional 7% of the retained C-6092 is removed during the second dewatering step.

It is believed that this simulation of the improved chemical addition method demonstrates the ability to significantly reduce the amount of unadsorbed chemical additive in the water of a paper manufacturing process while maintaining high chemical retention levels on the fiber fraction.

The foregoing detailed description has been for the purpose of illustration. Thus, a number of modifications and changes may be made without departing from the scope of the present invention. For instance, alternative or optional features described as part of one embodiment can be used to yield another embodiment. Additionally, two named components could represent portions of the same structure. Further, various alternative process and equipment arrangements may be employed, particularly with respect to the stock preparation; headbox, forming fabrics, web transfers, creping and drying. Therefore, the invention should not be limited by the specific embodiments described, but only by the claims.

## Claims

1. A method comprising:
creating a fiber slurry (20) comprising water, cellulosic fibers, and an adsorbable chemical additive;
**characterized in that** the adsorbable chemical additive is added to the slurry of water and cellulosic fibers in an amount of about 5 kilograms per metric ton or greater, and that the method further comprises the steps of:
dewatering the fiber slurry to remove unadsorbed chemical additive (24) and provide a thickened fibrous slurry; and
diluting the thickened fibrous slurry with fresh water (35).

2. The method of claim 1, wherein creating said fiber slurry comprises adding the adsorbable chemical additive to an aqueous solution comprising the water and cellulosic fibers.

3. The method of claim 1 or 2, wherein said fiber slurry has a consistency of 20 percent or lower, and preferably 5 percent or lower.

4. The method of any preceding claim, wherein the step of dewatering increases the consistency of the fiber slurry to about 30 percent or greater.

5. The method of any preceding claim, wherein the step of diluting the thickened fibrous slurry decreases the consistency of the thickened fiber slurry to about 5 percent or lower.

6. The method of any preceding claim, further comprising maintaining the removed unadsorbed chemical additive separate from the fiber slurry.

7. The method of any preceding claim, wherein the fresh water is completely free of unadsorbed chemical additive.

8. The method of any preceding claim, wherein sufficient residence time is provided after the chemical additive is added to allow for adsorption.

9. The method of any preceding claim, wherein the removed unadsorbed chemical additive is reused in a processing step prior to dewatering the fiber slurry.

10. The method of any preceding claim, wherein the adsorbable chemical additive comprises a debonding agent.

11. The method of any of claims 1 to 9, wherein the adsorbable chemical additive comprises a softening agent.

12. The method of any preceding claim, wherein the chemical additive comprises a debonding agent or softening agent and the fiber slurry is not subjected to high shear refining forces once the chemical additive is added to the fiber slurry.

13. The method of any preceding claim, wherein the diluted fiber slurry is treated with a second adsorbable chemical additive, dewatered a second time to remove unadsorbed chemical additives and diluted a second time.

14. The method of claim 13, wherein the second chemical additive comprises a softening agent.

15. The method of claim 13, wherein the second chemical additive comprises a debonding agent.

16. The method of any preceding claim, further comprising forming a paper product comprising a plurality of layers, with one but not all of the layers being formed from the fiber slurry containing the adsorbable chemical additive.

17. The method of claim 1 further comprising:
dewatering said fiber slurry comprising water, cellulosic fibers and the adsorbable chemical additive to a consistency of about 20 percent or greater;
passing the dewatered fiber slurry through a dispenser to mechanically work the fibers;
diluting the fiber slurry with fresh water that is substantially free of the first chemical additive to a consistency of about 5 percent or less;
adding a second adsorbable chemical additive comprising a debonding agent or a softening agent to the fiber slurry;
dewatering the fiber slurry to a consistency of about 20 percent or greater;
diluting the fiber slurry with fresh water that is substantially free of the second chemical additive to a consistency of about 5 percent or less; and
forming a paper product from the fiber slurry.

18. The method of claim 17, wherein the first chemical additive comprises a bonding agent.

19. The method of any preceding claim further comprising the steps of creating a second fiber slurry (26) that is substantially free of the adsorbable chemical additive; and
forming a paper product using a layered headbox, the first fiber slurry comprising said adsorbable chemical additive being supplied to a first headbox layer and the second fiber slurry being supplied to a second headbox layer.

20. The method of any preceding claim further comprising the step of forming a paper product having a chemical additive retention of about 4 kilograms per metric ton or greater.

21. The method of any of claims 1 to 19 further comprising the step of forming a paper product having a chemical additive retention of about 5 kilograms per metric ton or greater.

22. The method of claim 21, wherein said product comprises a central layer consisting essentially of softwood fibers and two outer layers comprising about 70 percent or greater hardwood fibers.

## Patentansprüche

1. Ein Verfahren, welches umfasst:
Erzeugen eines Faserbreis (20), welcher Wasser, zellulosische Fasern und ein adsorbierbares chemisches Additiv umfasst;
**dadurch gekennzeichnet, dass** das adsorbierbare chemische Additiv zu dem Brei aus Wasser und zellulosischen Fasern in einer Menge von ungefähr 5 Kilogramm pro metrischer Tonne oder mehr zugegeben wird, und dass das Verfahren des Weiteren die Schritte umfasst:
Entwässern des Faserbreis, um nicht-adsorbiertes chemisches Additiv (24) zu entfernen und einen verdickten faserigen Brei bereitzustellen; und
Verdünnen des verdickten faserigen Breis mit Frischwasser (35).

2. Das Verfahren gemäß Anspruch 1, wobei das Erzeugen des Faserbreis das Hinzugeben des adsorbierbaren chemischen Additivs zu einer wässrigen Lösung umfasst, welche das Wasser und zellulosische Fasern umfasst.

3. Das Verfahren gemäß Anspruch 1 oder 2, wobei der Faserbrei eine Konsistenz von 20 Prozent oder weniger aufweist, und vorzugsweise 5 Prozent oder weniger.

4. Das Verfahren gemäß einem der vorherigen Ansprüche, wobei der Schritt des Entwässerns die Konsistenz des Faserbreis bis ungefähr 30 Prozent oder mehr erhöht.

5. Das Verfahren gemäß einem der vorherigen Ansprüche, wobei der Schritt des Verdünnens des verdickten faserigen Breis die Konsistenz des verdickten Faserbreis bis ungefähr 5 Prozent oder geringer erniedrigt.

6. Das Verfahren gemäß einem der vorherigen Ansprüche, welches des Weiteren das Aufbewahren des entfernten unadsorbierten chemischen Additivs getrennt von dem Faserbrei umfasst.

7. Das Verfahren gemäß einem der vorherigen Ansprüche, wobei das Frischwasser gänzlich frei von unadsorbiertem chemischem Additiv ist.

8. Das Verfahren gemäß einem der vorherigen Ansprüche, wobei genügend Einwirkzeit zur Adsorption gewährt wird nachdem das chemische Additiv hinzugegeben wurde.

9. Das Verfahren gemäß einem der vorherigen Ansprüche, wobei das entfernte unadsorbierte chemische Additiv in einem Verfahrensschritt vor dem Entwässern des Faserbreis wiederverwendet wird.

10. Das Verfahren gemäß einem der vorherigen Ansprüche, wobei das adsorbierbare chemische Additiv ein Debonding-Mittel umfasst.

11. Das Verfahren gemäß einem der Ansprüche 1 bis 9, wobei das adsorbierbare chemische Additiv einen Weichmacher umfasst.

12. Das Verfahren gemäß einem der vorherigen Ansprüche, wobei das chemische Additiv ein Debonding-Mittel oder einen Weichmacher umfasst und wobei der Faserbrei nicht hohen Refiner-Scherkräften ausgesetzt ist sobald das chemische Additiv zum Faserbrei hinzugegeben wurde.

13. Das Verfahren gemäß einem der vorherigen Ansprüche, wobei der verdünnte Faserbrei mit einem zweiten adsorbierbaren chemischen Additiv behandelt wird, ein zweites Mal entwässert wird, um unadsorbierte chemische Additive zu entfernen, und ein zweites Mal verdünnt wird.

14. Das Verfahren gemäß Anspruch 13, wobei das zweite chemische Additiv einen Weichmacher umfasst.

15. Das Verfahren gemäß Anspruch 13, wobei das zweite chemische Additiv ein Debonding-Mittel umfasst.

16. Das Verfahren gemäß einem der vorherigen Ansprüche, welches des Weiteren das Bilden eines Papierprodukts umfasst, welches eine Vielzahl an Schichten umfasst, wobei eine aber nicht alle der Schichten aus dem Faserbrei gebildet sind, der das adsorbierbare chemische Additiv enthält.

17. Das Verfahren gemäß Anspruch 1, welches des Weiteren umfasst:
Entwässern des Faserbreis, der Wasser, zellulosische Fasern und das adsorbierbare chemische Additiv umfasst, zu einer Konsistenz von ungefähr 20 Prozent oder mehr;
Führen des entwässerten Faserbreis durch einen Dispenser, um die Fasern mechanisch zu bearbeiten;
Verdünnen des Faserbreis mit Frischwasser, das im Wesentlichen frei ist von dem ersten chemischen Additiv bis zu einer Konsistenz von ungefähr 5 Prozent oder weniger;
Hinzugeben eines zweiten adsorbierbaren chemischen Additivs, welches ein Debonding-Mittel oder einen Weichmacher umfasst, zum Faserbrei;
Entwässern des Faserbreis bis zu einer Konsistenz von ungefähr 20 Prozent oder mehr;
Verdünnen des Faserbreis mit Frischwasser, das im Wesentlichen frei ist von dem zweiten chemischen Additiv bis zu einer Konsistenz von ungefähr 5 Prozent oder weniger; und
Bilden eines Papierprodukts aus dem Faserbrei.

18. Das Verfahren gemäß Anspruch 17, wobei das erste chemische Additiv ein Bindemittel umfasst.

19. Das Verfahren gemäß einem der vorherigen Ansprüche, welches des Weiteren die Schritte umfasst des Erzeugens eines zweiten Faserbreis (26), der im Wesentlichen frei ist von dem adsorbierbaren chemischen Additiv; und
Bilden eines Papierprodukts unter Verwendung eines in Lagen aufgebauten Auflaufkastens, wobei der erste Faserbrei, der das adsorbierbare chemische Additiv umfasst, einer ersten Auflaufkastenlage zugeführt wird, und wobei der zweite Faserbrei einer zweiten Auflaufkastenlage zugeführt wird.

20. Das Verfahren gemäß einem der vorherigen Ansprüche, welches des Weiteren den Schritt des Bildens eines Papierprodukts umfasst, welches ein Rückhaltevermögen für chemisches Additiv von ungefähr 4 Kilogramm pro metrischer Tonne oder mehr aufweist.

21. Das Verfahren gemäß einem der Ansprüche 1 bis 19, welches des Weiteren den Schritt des Bildens eines Papierprodukts umfasst, welches ein Rückhaltevermögen für chemisches Additiv von ungefähr 5 Kilogramm pro metrischer Tonne oder mehr aufweist.

22. Das Verfahren gemäß Anspruch 21, wobei das Produkt eine zentrale Schicht, welche im Wesentlichen aus Weichholzfasern besteht, und zwei äußere Schichten umfasst, welche ungefähr 70 Prozent oder mehr Hartholzfasern umfassen.

## Revendications

1. Procédé comprenant :
la création d'une bouillie de fibres (20) comprenant de l'eau, des fibres cellulosiques et un additif chimique adsorbable ;
**caractérisé en ce que** l'additif chimique adsorbable est ajouté à la bouillie d'eau et de fibres cellulosiques en une quantité d'environ 5 kg/tonne métrique ou plus, et **en ce que** le procédé comprend, en outre, les étapes suivantes :
l'extraction d'eau depuis la bouillie de fibres pour enlever l'additif chimique non-adsorbé (24) et aboutir à une bouillie fibreuse épaissie ; et
la dilution de la bouillie fibreuse épaissie avec de l'eau fraîche (35).

2. Procédé selon la revendication 1, dans lequel la création de la bouillie de fibres comprend l'ajout de l'additif chimique adsorbable à une solution aqueuse comprenant l'eau et les fibres cellulosiques.

3. Procédé selon la revendication 1 ou 2, dans lequel ladite bouillie de fibres a une concentration en fibres de 20 % ou moins, et de préférence de 5 % ou moins.

4. Procédé selon l'une quelconque des revendications précédentes, dans lequel l'étape d'extraction d'eau augmente la concentration en fibres de la bouillie de fibres jusqu'à environ 30 % ou plus.

5. Procédé selon l'une quelconque des revendications précédentes, dans lequel l'étape de dilution de la bouillie fibreuse épaissie réduit la concentration en fibres de la bouillie fibreuse épaissie jusqu'à environ 5 % ou moins.

6. Procédé selon l'une quelconque des revendications précédentes, comprenant, en outre, le fait de maintenir, séparé de la bouillie de fibres, de l'additif chimique non-adsorbé enlevé.

7. Procédé selon l'une quelconque des revendications précédentes, dans lequel l'eau fraîche est complètement dépourvue d'additif chimique non-adsorbé.

8. Procédé selon l'une quelconque des revendications précédentes, dans lequel un temps de séjour suffisant est prévu après ajout de l'additif chimique pour permettre l'adsorption.

9. Procédé selon l'une quelconque des revendications précédentes, dans lequel l'additif chimique non-adsorbé, enlevé, est réutilisé dans une étape de traitement antérieure à l'extraction d'eau de la bouillie de fibres.

10. Procédé selon l'une quelconque des revendications précédentes, dans lequel l'additif chimique adsorbable comprend un agent dé-liant.

11. Procédé selon l'une quelconque des revendications 1 à 9, dans lequel l'additif chimique adsorbable comprend un agent assouplissant.

12. Procédé selon l'une quelconque des revendications précédentes, dans lequel l'additif chimique comprend un agent dé-liant ou agent assouplissant et la bouillie de fibres n'est pas soumise à des forces d'affinage sous fort cisaillement une fois que l'additif chimique a été ajouté à la bouillie de fibres.

13. Procédé selon l'une quelconque des revendications précédentes, dans lequel la bouillie de fibres diluée est traitée avec un second additif chimique adsorbable, a son eau extraite une seconde fois pour enlever les additifs chimiques non-adsorbés et est diluée une seconde fois.

14. Procédé selon la revendication 13, dans lequel le second additif chimique comprend un agent assouplissant.

15. Procédé selon la revendication 13, dans lequel le second additif chimique comprend un agent dé-liant.

16. Procédé selon l'une quelconque des revendications précédentes, comprenant, en outre, la formation d'un produit en papier comprenant une pluralité de couches, une des couches, mais pas toutes, étant formée à partir de la bouillie de fibres contenant l'additif chimique adsorbable.

17. Procédé selon la revendication 1, comprenant en outre :
l'extraction d'eau depuis ladite bouillie de fibres comprenant de l'eau, des fibres cellulosiques et l'additif chimique adsorbable jusqu'à une concentration en fibres d'environ 20 % ou plus ;
le passage de la bouillie de fibres, de laquelle de l'eau a été extraite, au travers d'un distributeur pour travailler mécaniquement les fibres ;
la dilution de la bouillie de fibres avec de l'eau fraîche qui est sensiblement dépourvue du premier additif chimique jusqu'à une concentration en fibres d'environ 5 % ou moins ;
l'ajout d'un second additif chimique adsorbable comprenant un agent dé-liant ou agent assouplissant à la bouillie de fibres ;
l'extraction d'eau depuis la bouillie de fibres jusqu'à une concentration en fibres d'environ 20 % ou plus ;
la dilution de la bouillie de fibres avec de l'eau fraîche qui est sensiblement dépourvue du second additif chimique jusqu'à une concentration en fibres d'environ 5 % ou moins ; et
la formation d'un produit en papier à partir de la bouillie de fibres.

18. Procédé selon la revendication 17, dans lequel le premier additif chimique comprend un agent dé-liant.

19. Procédé selon l'une quelconque des revendications précédentes, comprenant, en outre, les étapes suivantes
la création d'une seconde bouillie de fibres (26) qui est sensiblement dépourvue d'additif chimique adsorbable ; et
la formation d'un produit en papier en utilisant une caisse de tête à étages, la première bouillie de fibres qui comprend ledit additif chimique adsorbable étant fournie à une première caisse de tête et la seconde bouillie de fibres étant fournie à une seconde caisse de tête.

20. Procédé selon l'une quelconque des revendications précédentes, comprenant, en outre, l'étape de formation d'un produit en papier ayant une rétention de l'additif chimique d'environ 4 kg/tonne métrique ou plus.

21. Procédé selon l'une quelconque des revendications 1 à 19, comprenant, en outre, l'étape de formation d'un produit en papier ayant une rétention de l'additif chimique d'environ 5 kg/tonne métrique ou plus.

22. Procédé selon la revendication 21, dans lequel ledit produit comprend une couche centrale consistant essentiellement en fibres de résineux et deux couches extérieures comprenant environ 70 % ou plus de fibres de feuillus.
